

## UNITED STATES PATENT OFFICE

2,121,151

OIL FOR WITHSTANDING HIGH BEARING  
PRESSURES AND METHOD OF MAKING  
THE SAMECharles B. Karns, Pittsburgh, Pa., assignor to  
Standard Oil Development Company, a corpo-  
ration of DelawareNo Drawing. Application May 2, 1934,  
Serial No. 723,505

20 Claims. (Cl. 87—9)

The present invention relates to improved lubricating oils, especially to oils of high quality and capable of withstanding high bearing pressures. The invention will be fully understood 5 from the following description.

Leaded or lead-containing oils have been used for a considerable period of time because of their ability to withstand heavy loads and lead oleate is the most generally used substance employed in 10 their manufacture. Unfortunately, lead oleate and the lead salts of most of the similar fatty acids are not freely soluble in high grade lubricating oil bases, such as cylinder oils, bright stocks and the like, derived from wax bearing crudes. 15 On standing for a relatively short time the lead compound is observed to settle from the oil in a thick sludge. The lower grade base oils, however, are capable of maintaining the oil in a stable form and it is for this reason that such 20 low grade base oils are used in the manufacture of leaded lubricants.

The low grade base oils which are ordinarily used in making up leaded lubricants are generally characterized by a Viscosity Index of 50 or 25 below, see Davis and Dean, Chemical and Metallurgical Engineering 36-618 (1929) for a definition of the term "Viscosity Index." It is true that asphalt containing residual oils such as black 30 oils of somewhat higher Viscosity Index than 50 have been used, but in all cases it is believed that whether distillate or residual, the base oils used for the manufacture of leaded lubricants are ordinarily characterized by Viscosity Indices below 35 80. Such oils are ordinarily derived from naphthenic or asphalt base crudes and not from the higher grade crudes such as are characterized by the presence of wax.

The present invention relates to a lubricating oil containing a high grade base which is capable 40 of maintaining the leaded compound in a stable form. The base oil used in the present invention, which is normally incapable of holding the leaded compound in solution, is characterized by having the Viscosity Index above 60 for distillates and above 80 for residual oils free from 45 asphalt and may have a Viscosity Index of 85, 90, or even higher. It is possible to produce stable, light colored, clean and transparent oils containing lead in effective quantities from oils of Pennsylvania quality or even better, such as the hydrogenated petroleum oils, and the high grade oils 50 produced from solvent extraction processes, and even from synthetic oils produced by condensation of cracked or dehydrogenated wax, either alone or condensed with aromatic hydrocarbons,

and which may be characterized by Viscosity Indices well above 100.

The oil which is selected for the present purpose should be of good color and well refined. Its viscosity may vary considerably, depending upon the service for which the oil is destined. For some purposes a viscosity from 50 to 60 seconds Saybolt at 210° F. to 80 or 90 is satisfactory, but for gear or transmission oils for heavier service higher viscosities are desirable, say above 10 100 or 120 at 210° F., and they may be as high as 200 or 250 for particularly heavy duty. The base oil is first subjected to a mild oxidation treatment which is preferably carried out by bubbling air or other oxidizing gas through the 15 oil, while maintained at a temperature of the order of 400 to 450° F. The time required for the treatment depends on the temperature and the rate of air flow, and the conditions may be interadjusted with ease so as to obtain products 20 to which the lead may be added in a stable form. To illustrate the conditions which might be used, it is found that at a temperature of 450° F. air 25 may be bubbled through 3 gallons of oil at a rate of about 2 cu. ft. per hour for a time of approximately 2½ hours. These conditions vary considerably for different stocks. At the end of this time the other ingredients of the compound are added and it is found that they are capable of remaining in the compound in a stable form. The 30 oxidation required is very mild and the chemical effect is not clearly known. While oxidation with air or oxygen is preferred other oxidizing agents may be used and it is not necessary to treat the entire base oil, in fact only a portion need be so 35 treated and later added to the bulk, nor is it necessary that the oil treated be a portion of the base stock itself.

One of the constituents added to the base is, of course, the lead soap or salt, and it is preferred 40 to use lead oleate, which is the most widely available substance of the type. Other lead compounds, of course, may be used, such as the lead soaps of other fatty acids, stearate, palmitate, ricinoleate, resinate or other soap normally insoluble in the high quality base. The lead soap is ordinarily added in proportion below about 10% of the oil; for example, it may be within the range of 5 to 15%, or, as expressed in terms of metallic lead, from 1 to 3%.

A sulfurizing agent is also added to the compound to make the product effective in carrying heavy loads. The sulfurizing agent is preferably of the "corrosive" type, by which is meant that it is of the class of sulfur compound capable of dis-

coloring a bright copper strip when allowed to stand in the liquid for several hours at 212° F. according to the general conditions of the A. S. T. M. corrosion test. It will be understood that 5 non-corrosive sulfur compounds may be used, but the corrosive type is so much preferable for the present purposes that they should always be used where possible. Among the corrosive substances may be mentioned free sulfur and compounds such as occur in the lower grade crudes 10 rich in sulfur and its compounds. Various synthetic materials may also be used particularly those heavy enough not to be lost on heating, such as animal, vegetable and marine oils, sulfurized by the action of free sulfur at elevated 15 temperatures, and the products of reaction of these materials with other known sulfurizing agents. Synthetic materials may be produced by first halogenating fatty oils, fats and waxes, such as paraffin wax, and then reacting the halogenated product or after dehalogenation, with an 20 inorganic sulfur compound, such as a sulfide, hydrosulfide, various polysulfides of alkali and alkaline earth metals. The reaction is readily 25 accomplished at about 200 to 300° F. and the sulfur gradually replaces the chlorine or other halogen.

The various sulfur compounds mentioned above 30 are to be considered merely as illustrations of the type of sulfurizing agents that may be employed. They are added to the oil so as to furnish about 1/2 to 5% of sulfur. The sulfurizing agent may be added along with the lead compound or they may be added separately, or the sulfur compound 35 may be added to the oil prior to the mild oxidation treatment referred to above.

By the above methods it is possible to produce 40 leaded oils of higher quality than are previously known, in that it is possible to use bright stocks and cylinder oils derived from the finest crude sources. It is sometimes observed that the Viscosity Index of the finished compound is less than that of the base added and this is due to the effect 45 of the particular sulfur compound added, but it is also possible to select sulfur compounds which show little or no effect on the Viscosity Index and in this case products with an index of 80 to 90 or even higher can be readily produced. These compounds are capable of withstanding the highest bearing pressures ordinarily encountered with 50 low friction, without excess temperature rise and with smooth friction-load curves.

The following examples are presented to illustrate the method of producing compounded oils 55 according to the present invention and of their properties.

#### Example I

The oil base selected was a heavy Pennsylvania cylinder oil, bright stock, having a viscosity 60 of sec. Saybolt at 210° F. and 100 VI. Three gallons of this stock is mildly oxidized by blowing air thru while at 450° F. for about 2 1/2 hours. The oil became slightly more viscous but did not change substantially in appearance. To the 65 oil is added 1% of flowers of sulfur and the oil was held at 400° for about half an hour while agitated. The product is then cooled and 10% of lead oleate gradually incorporated.

The final product is of excellent appearance, 70 only a few shades darker than the original oil. When tested on the Almen machine, described in Automotive Industries 11/19/32 vol. 67 No. 22, page 650, it was capable of carrying the full load of 15,000 lbs. and the friction curve was smooth. 75 The final value of friction was 32 pound feet.

This oil was stable while similar oils made up with the untreated oil quickly settled out.

#### Example II

A Pennsylvania steam refined cylinder oil was 5 incorporated with 10% of lead oleate and the mixture blown with air at 450° F. for about 2 hours, the rate being about the same as in the previous example. To the mixture is added 1% 10 of sulfurized pine oil, so that the final blend contained 3% of corrosive sulfur.

This oil was of good appearance and stable and 15 on the Almen machine showed about the same result as the oil of Example I.

The present invention is not to be limited by 15 any theory of the mechanism of the oxidation step or to any particular sulfur compound or ingredient but only to the following claims.

I claim:

1. A method for producing improved lubricating 20 oils comprising, subjecting a high quality lubricating oil base to mild oxidation to increase its solvency for lead soaps and adding a lead soap and then a sulfurizing agent uncombined with the lead of the lead soap.

2. An improved lubricating oil comprising a 25 lubricating oil which has been mildly oxidized by blowing with an oxygen containing gas, free from asphalt and characterized by a Viscosity Index above about 50, a lead soap and a sulfurizing agent uncombined with the lead of the lead soap.

3. An improved lubricating oil comprising a 30 base oil having a Viscosity Index above 80 and a viscosity above about 50 seconds Saybolt at 210° F., lead oleate and corrosive sulfur uncombined with lead of the lead soap, the base having been mildly oxidized while at about 450° F. with an oxygen containing gas only to such a degree as to render the finished oil stable.

4. An improved lubricating oil comprising a 35 base oil having a Viscosity Index above about 80 and a viscosity above about 100 seconds Saybolt at 210° F., lead oleate in proportion of about 40 5 to 15%, and corrosive sulfur in proportion from about 1/2 to 5% uncombined with the lead of the lead soap, the base oil being mildly oxidized at a temperature of the order of 400 to 450° F. by blowing with an oxygen containing gas for a time sufficient only to render the finished compound stable.

5. A method for producing improved lubricating 45 oils comprising, mildly oxidizing a lubricating oil of Viscosity Index above about 50 with air to such a degree as to maintain a lead soap in stable form, and adding to the oil 5 to 15% of a lead soap and an organic sulfurizing agent uncombined with the lead of the lead soap in an amount sufficient to furnish 1/2 to 5% of sulphur.

6. A method for producing an improved high 50 pressure bearing lubricating oil comprising subjecting a petroleum lubricating oil base characterized by a Viscosity Index above 80 to a mild oxidation treatment at a temperature of the order of 400 to 450° F. and for such time as to adapt it to maintain lead oleate in a stable form, adding 60 to the oil 5 to 15% of lead oleate and 1/2 to 5% of corrosive sulfur uncombined with the lead of the lead soap.

7. Process of manufacturing an improved 65 lubricating oil comprising adding to a base oil having a Viscosity Index above 80 and a viscosity above 50 seconds Saybolt at 210° F., which has been mildly oxidized at about 450° F. with an oxygen containing gas only to such a degree as to render the finished oil stable, free sulfur and 70 75

- holding the mixture for a prolonged period at a reaction temperature to permit reaction between the sulfur and the oil, followed by the addition thereto of a lead soap.
8. Process of manufacturing an improved lubricating oil comprising adding to a base oil having a Viscosity Index above about 80 and a viscosity above about 100 seconds Saybolt at 210° F., which has been mildly oxidized at a temperature of the order of 400 to 450° F. by blowing with oxygen containing gas for a time sufficient only to render the finished oil stable, free sulfur in the proportion of about  $\frac{1}{2}$  to 5% and holding the mixture for a prolonged period at a reaction temperature to permit reaction between the sulfur and the oil, followed by the addition thereto of 5 to 15% of lead oleate.
9. An improved lubricating oil comprising a refined base oil distillate having a Viscosity Index above 60 which has been mildly oxidized by blowing with an oxygen containing gas, a lead soap soluble therein and a minor quantity of a substance selected from the class consisting of free sulfur and sulfur compounds of mineral, vegetable and animal oils.
10. A composition in accordance with claim 9 in which said lead soap is present in the proportion of from 5 to 15%.
11. A composition in accordance with claim 9 in which said lead soap is present in the proportion of from 5 to 15% and said substance selected from the class consisting of free sulfur and sulfur compounds of mineral, vegetable and animal oils is present in an amount sufficient to furnish  $\frac{1}{2}$  to 5% of sulfur.
12. An improved lubricating oil comprising a residual oil free from asphalts having a Viscosity Index above 80 which has been subjected to mild oxidation by blowing with an oxygen containing gas, a lead soap and a substance selected from the class consisting of free sulfur and sulfur compounds of mineral, vegetable and animal oils.
13. A composition in accordance with claim 12 in which said lead soap is present in the proportion of from 5 to 15%.
14. A composition in accordance with claim 12 in which said lead soap is present in the proportion of from 5 to 15% and said substance selected from the class consisting of free sulfur and sulfur compounds of mineral, vegetable and animal oils is present in an amount sufficient to furnish from  $\frac{1}{2}$  to 5% of sulphur.
15. An improved stable composition comprising a refined base oil having a Viscosity Index above 50, which has been subjected to mild oxidation to increase the solvency of the oil for lead soaps, said base oils previous to oxidation being partial or non-solvents for lead soaps, and a lead soap dissolved therein.
16. Composition in accordance with claim 15 in which said lead soap dissolved therein is lead oleate in the proportion of from about 5 to 15%.
17. Process for producing a stable lubricating oil lead soap composition comprising mildly oxidizing high grade lubricating oils which are partial or non-solvents for lead soaps and are characterized by Viscosity Indexes above about 50 by blowing with an oxygen containing gas, and dissolving therein a lead soap.
18. Process in accordance with claim 17 in which said lead soap dissolved in the oxidized high grade lubricating oil is lead oleate in the proportion from about 5 to 15%.
19. An improved stable composition comprising a refined base oil of the class consisting of distillates having Viscosity Indexes above 60 and residual oils free from asphalts having Viscosity Indexes above 80 which have been mildly oxidized by blowing with an oxygen containing gas, and a lead soap.
20. Composition in accordance with claim 19 in which said lead soap is from about 5 to 15% of lead oleate.

CHARLES B. KARNS.